

Feb. 17, 1925.

1,526,513

L. F. J. C. A. THIBAUDIER ET AL  
PROCESS AND APPARATUS FOR THE THERMIC TREATMENT OF STEELS AND  
IN GENERAL OF ALL OTHER ALLOYS SUSCEPTIBLE OF HARDENING  
Filed Dec. 15, 1921

2 Sheets-Sheet 1

Fig. 1



Fig. 2



Fig. 3



Fig. 4



Inventors  
L. F. J. C. A. Thibaudier  
H. Viteaux  
By Marks Clark  
Atty's.

Feb. 17, 1925.

1,526,513

L. F. J. C. A. THIBAUDIER ET AL  
PROCESS AND APPARATUS FOR THE THERMIC TREATMENT OF STEELS AND  
IN GENERAL OF ALL OTHER ALLOYS SUSCEPTIBLE OF HARDENING  
Filed Dec. 15, 1921

2 Sheets-Sheet 2

Cooling-diagram of a Rail

fig. 5



Inventors  
L.F.J.C.A. Thibaudier  
H. Viteau  
By Marks Clark Atys.

Patented Feb. 17, 1925.

1,526,513

# UNITED STATES PATENT OFFICE.

LOUIS FRANÇOIS JOSEPH CLAUDE ANTOINE THIBAUDIER AND HENRI VITEAUX, OF PARIS, FRANCE.

PROCESS AND APPARATUS FOR THE THERMIC TREATMENT OF STEELS AND IN GENERAL OF ALL OTHER ALLOYS SUSCEPTIBLE OF HARDENING.

Application filed December 15, 1921. Serial No. 522,637.

To all whom it may concern:

Be it known that we, LOUIS FRANÇOIS JOSEPH CLAUDE ANTOINE THIBAUDIER and HENRI VITEAUX, citizens of the Republic of France, and residing at Paris, Seine Department, No. 19 Rue de la Rochefoucauld, in the Republic of France, have invented a certain new and useful Process and Apparatus for the Thermic Treatment of Steels and in General of all other Alloys Susceptible of Hardening, of which the following is the specification.

The thermic treatment of metallurgical products is recognized to afford a considerable number of advantages, and such treatment will give rise to marked improvements in the mechanical properties of products of this class. This treatment which comprises in general a reheating operation followed by 15 hardening, then a second reheating or annealing, has not however been adapted in current practice to the extent which it would appear to merit, for in fact in a considerable number of cases it is recognized that 20 the operations required for the treatment, and especially for the reheating before or after the hardening, are too difficult to carry into effect or will require an excessive outlay.

30 In order to simplify these operations and more particularly to obviate the annealing after hardening it has been proposed to arrest the hardening before the said products have become entirely cooled, or on the other 35 hand to carry out the hardening operation in a limited volume of liquid. In the first case, the quantity of heat remaining in the piece after the hardening is stopped is sufficient to reheat the hardened parts and to 40 afford the annealing, and in the second case, the heating of the hardening bath, whose mass is made proportional to the mass of the piece to be treated, will reduce the rate of heating and will afford a slow hardening 45 which is adapted to produce similar results to those which would be obtained by a more energetic hardening with subsequent annealing.

These simplified methods of treatment 50 have not come into general use to the extent which might be supposed, by reason of the serious inconveniences which they present. In the first-mentioned process, the rate of cooling of the surfaces in contact

with a considerable volume of liquid is so 55 high that in order to obtain certain and regular results it would be necessary to arrest the hardening after a stated time within one second, but such exact operations are very difficult to carry out in usual shop 60 practice, whence it will follow that the results afforded by this method of treatment will have an uncertain and irregular character. On the other hand it becomes difficult with this method to carry out the hardening of the pieces to any great depth without an undue cooling of the surfaces, and the latter will thereby remain in a hard 65 and brittle condition.

The method of hardening in a quantity 70 of liquid proportional to the mass under treatment will permit of reducing the rate of cooling and will thus facilitate to determine the instant of stopping the tempering operation in order to obtain a given hardness. But it is recognized by numerous experimenters that the said process gave rise 75 to a very irregular hardening not only between the various pieces but even throughout the mass of a single piece. Furthermore, 80 and doubtless by reason of this lack of homogeneity and the consequent internal stresses, the pieces treated in this manner are much subject to developing interior 85 cracks.

The difficulties in the use of the above methods are due to the following circumstances: 1—The rate of cooling of the surfaces immersed in a considerable volume of cold liquid is large. 2—The rapid heating 90 of a limited mass of liquid and the formation of bubbles of vapor within the said mass will constitute very irregular phenomena.

This invention consists in submitting the pieces under treatment and employed at a 95 temperature above the critical temperature, to a stated number of short immersions in water or like liquid in the hot or cold state which is provided in a limited quantity and in proportion to the size of the said pieces. 100 Experience shows that it will now be possible to entirely obviate above-mentioned drawbacks while at the same time retaining the advantages of a partial hardening as well as of a hardening in a reduced volume of liquid. 105 The quantity of liquid to be used, duration of the immersion and emersion, and the number of these latter operations, are to be de-

terminated by experience according to the size of the pieces under treatment and the results to be obtained in such manner that the said pieces shall be cooled from their initial temperature—which is above the critical temperature—to the temperature of the atmosphere according to a law of variation of temperatures which is intermediate between the law of variation of temperatures corresponding to the integral cooling in a large volume of water and the law of variation of temperatures corresponding to the cooling in the open air, the said law being of such character as to afford the modifications of structure corresponding to the properties which it is desired to obtain, in a single operation, by the thermic treatment.

By "law of variation of temperatures", we mean the connection existing between the intervals of time and the successive temperatures through which passes a body which is submitted to a determined cooling process. This law of variation can be materialized and expressed by a curve if we register the successive temperatures corresponding to the known intervals of time and if on a diaphragm the times are indicated by abscissæ and the temperatures by ordinates, one of the figures of the drawing annexed by way of example indicates curves about cooling in water, in open air, and according to the process forming the subject-matter of the present invention.

The duration of the immersion and the volume of liquid used for the hardening bath are preferably determined in such manner that the bars or like pieces to be treated shall be permitted to cool in a sufficiently rapid manner to cover the stipulated time without however permitting the speed of cooling to attain the value above which interior or exterior cracking effects are to be apprehended. The time required for the emersion period is of sufficient length in order that during each of the said periods there will be produced an equalization of the temperature in the tempered regions. The number of immersions is also chosen in such manner that the quantity of heat remaining in the mass of the said pieces after the last immersion is susceptible of heating the hardened parts to a temperature below the critical point but still sufficient to effect the desired annealing operation. In some cases it will not be necessary to effect the complete emersion of the pieces under treatment. On the other hand it may be found preferable in certain cases to vary the depths or heights of immersion and emersion during the treatment.

60 The said method of operation will afford the following advantages:

1. During each immersion, the surface portions of the pieces under treatment which have become tempered during the preceding immersion, are now slowly cooled by the air,

whereas they are highly heated by the heat coming from the centre of the said pieces. In consequence, it will be possible, by suitably regulating on the one hand the number and the relative duration of immersions and emersions and on the other hand the volume of the hardening bath, to carry into effect in the parts to be treated a law of temperature variation which shall be intermediate between the cooling in cold or more or less hot water and the cooling in the open air, and to confer upon the said parts in a single operation the mechanical properties corresponding to the said law of cooling.

2. The emersions increase the duration of the treatment and also reduce the rate of cooling, and in consequence it becomes an easy matter to determine the exact moment for arresting the treatment in order to obtain a given result.

3. The reheating obtained during each emersion will act to neutralize in the tempered regions the inequalities of temperature resulting from the differences in cooling which may have been produced during the preceding immersion, the vapor bubbles formed within the liquid will disappear, and the bath which is stirred by the immersion and removal of the pieces will assume a more uniform temperature, whence it will follow that by reason of the separate and successive hardening operations there will be obtained results of an absolutely regular character in any given piece of work and between the various pieces of work, at the same time obviating interior cracks which would tend to produce inequalities in the cooling.

4. For the same pieces to be treated and the same hardening bath, the heating of the said bath is more rapid as the initial temperature of the pieces is higher. This effect will compensate in a certain measure any differences of temperature between the pieces before the treatment and will permit for instance to obtain substantially identical results by using the present process, without any reheating, for the treatment of bars leaving the rolls at temperatures above the critical point but differing among themselves by 25 to 50° centigrade.

It will be possible to determine in advance and for all cases the number and the duration of the immersions and the quantity of liquid to be used for the hardening bath, since these data will vary with the size of the pieces under treatment and the properties which is proposed to give to the same. But the determination of the various factors used in the process may be carried out with facility by making a few previous tests whose results are checked by mechanical and micrographic tests. An example of the use of the said process will be described in detail hereunder.

The said invention is applicable in a gen-

eral manner to the thermic treatment of all pieces of carbon steel or special steel or like alloys susceptible of hardening which are to be treated in the whole piece or in a 5 certain portion thereof; but special mention will be made of the application of the said process to the thermic treatment of rails of carbon steel, with a description of the operating method employed and of an apparatus 10 for the hardening of the rails by successive immersions and emersions.

For a long time past, a thermic treatment of railway or tramway rails has been recommended which would have the effect of increasing 15 the hardness of the rail to a considerable degree, thus increasing the resistance to the wear of the rail head to a depth of 15 or 20 millimetres below the rolling surface without appreciably modifying the other 20 properties of the metal, and particularly without rendering it brittle. By the use of the present hardening process and apparatus as described hereunder, the desired treatment can be given with great facility to bars of all 25 desired lengths which are operated upon directly after leaving the rolling mill.

The following description together with the accompanying drawings which are given by way of example show embodiments of 30 this invention, wherein:

Fig. 1 is an elevational view of one form of construction of the apparatus.

Fig. 2 is a cross-section of the same.

Figs. 3 and 4 show in like manner a modified form of construction of the said apparatus.

Fig. 5 shows curves regarding the cooling of a rail in water, in open air and according to the process forming the subject 40 matter of the present invention.

The apparatus comprises a horizontal beam *a* supporting by means of the brackets *b* the roller *c* whereupon are caused to bear the flanges or in the case of double-headed rails 45 the bottom part of the rails under treatment. Below the beam *a* is disposed a small tank *d* containing a determined quantity of cold water which is calculated according to the section of the rail and which is renewed after 50 the treatment of each bar. The rails leaving the rolls at a temperature of 800-850° centigrade are suspended by the flange from the beam *a* in such manner as to leave the head of the rail entirely free, as shown in Figs. 2 and 4. The head is then immersed 55 in the water to a depth which varies with the section and is given a series of immersions which are determined by experiment according to the cross-section and the weight 60 per linear metre of the rail under treatment.

By way of example, for a railway rail of the T-rail type weighing 45 kilograms per linear meter, the weight of the water employed 65 will be 10 kilogrammes per meter

and the number of immersions will be 15 per minute. After the requisite number of immersions, the rail is removed for the last time from the water, lifted out of the apparatus and placed upon a rack where it 70 becomes slowly cooled off in the open air.

When the hardening operation is completed, the water in the tank, which has reached a temperature of 90 to 95° centigrade is rapidly drawn off and is replaced 75 by cold water, and the apparatus is now ready for the treatment of a new piece. In order that the hardening operation shall afford regular results throughout the whole length of the rail, it is essential that the beam *a* and the rails themselves shall remain in a perfectly horizontal position during the entire treatment. To this effect the beam *a* is calculated in such manner as to support without appreciable deflection the 80 weight of the heaviest rails under the treatment; the brackets *b* are also given a sufficient length in order that the quantities of heat transmitted from the rails to the beam by conduction and by radiation shall not 85 cause the deformation of the said beam. For the same purpose, heat insulating material is interposed between the rollers and the brackets, and also under the beam itself. If these precautions prove to be insufficient 90 for an active use of the apparatus, the said beam may be cooled by water circulation or by like means.

To obviate the deformation of the rails 100 themselves, which would tend to assume a curved shape under the action of the hardening operation, the apparatus may be provided for instance with roller carrying brackets *e* disposed along the said beam for securing the rails in the horizontal position 105 after placing the same in the apparatus and for limiting the deformation to the very small deflection which may take place between one of the said rollers and the adjacent roller carrying bracket *e*.

In the form of construction shown in Figs. 1 and 2, the beam *a* is stationary and the tank *b* is movable in the vertical sense by means of a suitable mechanical device.

In the second form of construction shown 115 in Figs. 3 and 4, the tank *b* is now stationary and the beam *a* is given an alternative vertical movement.

The invention is not limited to the two forms of construction as hereinbefore set 120 forth. The same results may in fact be obtained for instance by producing successive variations in the level of the hardening liquid in the said tank, with the tank and the rail both secured in the stationary position, and if desired the liquid will not be obliged to entirely leave contact with the bar to be treated.

Claims:

1. Process for the thermic treatment of 125

- objects having an elongated shape in steel or other alloys capable of being hardened, these objects being taken at a temperature which is higher than the critical one and being partially hardened in a bath, consisting in effecting the hardening through several immersions and emersions of short duration of the object to be treated and this in a bath of a determined volume.
10. 2. Process for the thermic treatment of articles made of steel or other alloys capable of being hardened and having an elongated shape, consisting in immersing several times in a limited quantity of hardening liquid and for a short period at every operation and over their whole length at each time the articles which have been previously heated above the critical point and in leaving these articles cool in the air for a few moments in the intervals between immersions, the duration of the immersions and emersions being such that the gradual lowering of the temperature of the articles will be in accordance, in proportion to the time, with a predetermined selected law.
3. A process for the treatment of rolled rails consisting in the act of taking the rail upon leaving the rolls, suspending the same with the rail head downward above a tank containing a hardening liquid, submitting the rail head to a succession of immersions in the said liquid, separated by emersions, and finally removing the rail from the liquid

and allowing it to cool slowly in the open air.

4. An apparatus for the thermic treatment of steel rails comprising a horizontal beam, rollers suspended in pairs below the said beam, a tank containing a hardening liquid and means for alternately raising and lowering the said beam, the rollers being spaced apart in such manner that the rail under treatment with the head downward is enabled to pass between the said rollers and to rest thereupon by the rail flange.

5. In an apparatus for the thermic treatment of rails, the combination of a beam, rollers suspended therefrom and adapted to support the flanges of the rail under treatment, rollers suspended from the beam and located in the intervals between the first rollers, these second rollers being adapted for maintaining the rail in a rigid position upon the first rollers, and a tank disposed below the said beam and containing a hardening liquid.

In testimony, that we claim the foregoing as our invention, we have signed our names in presence of two subscribing witnesses.

LOUIS FRANÇOIS JOSEPH CLAUDE  
ANTOINE THIBAUDIER.

HENRI VITEAUX.  
Witnesses:  
JOHN F. SIMONS,  
MAURICE ROUX.